

## UNITED STATES PATENT OFFICE

1,989,209

METHOD OF TREATING FABRICS AND  
COMPOSITION THEREFOR

Winfred Maxwell Mitchell, Hopewell, Va., and  
Henri Louis Barthelemy, Rome, Ga., assignors  
to Tubize Chatillon Corporation, New York,  
N. Y., a corporation of Delaware

No Drawing. Application November 2, 1933,  
Serial No. 696,448

## 4 Claims. (CL 28—1)

This invention relates to a method of treating woven, knitted or other textile fabrics made from or containing cellulose acetate to produce effects or patterns or otherwise modify the appearance 5 of the fabric.

It is the object of the invention to provide a method and compositions for use in practising the method whereby desired and novel effects may be produced in fabrics of the character described by modifying the appearance of selected 10 portions of such fabrics.

Other objects and advantages of the invention will be better understood by reference to the following specification in which the preferred embodiments of the invention are described.

The invention depends upon the effect of terpineol and products containing terpineol, such as pine oil or camphor oil, upon cellulose acetate. Terpineol is not a solvent for and, so far as is 20 known, does not react with cellulose acetate. It nevertheless has the property, when applied under suitable conditions, of delustering cellulose acetate and thereby modifying its appearance. When, therefore, terpineol and products containing it are applied to fabrics consisting of or including cellulose acetate, various effects, designs, or patterns may be developed to impart to the fabric a modified and desirable appearance.

In carrying out the invention, we prefer to utilize suitable pastes which can be applied to the fabric by printing, stamping, stenciling or similar operation. Such pastes may include, in addition to terpineol or products containing terpineol, suitable agents to afford body and adhesive qualities such, for example, as starches and gums, and suitable agents such as water to afford fluidity.

Such a composition may be applied to the fabric, preferably a lustrous cellulose acetate material, in any suitable manner to delineate or represent various patterns or designs. The goods carrying the impression are then subjected before drying to the action of steam at a suitable temperature and for a period sufficient to develop the pattern on the fabric. When the steaming is completed, the goods may be scoured, rinsed and finished in the ordinary way.

The temperature of the steam employed may be 212° F. or higher. The time required for steaming will vary depending upon the nature of the fabric. Usually about 30 minutes is sufficient to develop the pattern on the fabric. Those portions to which the composition has been applied will present a chalky appearance in contrast with the luster of the portions not treated.

The goods may be dyed before or after treat-

ment, suitable dyes adapted for cellulose acetate fabrics being used for that purpose. Those portions which are delustered by the procedure described will present a different appearance from the remaining portions, and beautiful and striking effects are thus produced on the fabric. 5

Mixed fabrics, including textile fibres other than cellulose acetate, may be treated similarly. Since only the cellulose acetate fibres are affected to any material extent by the treatment, various 10 effects may be achieved by the judicious combination of fibres and the application of the method to fabrics thus prepared.

As an example of a composition suitable for use in practice of the invention, the following is suggested:

|                  | Parts |
|------------------|-------|
| Starch           | 15    |
| Water            | 45    |
| Gum tragacanth   | 20    |
| Pine oil mixture | 20    |

The pine oil mixture may comprise:

|              | Percent |
|--------------|---------|
| Pine oil     | 70      |
| Monopole oil | 15      |
| Caustic soda | 15      |

The composition as described affords a paste suitable for application to fabrics. When fabrics to which the paste has been applied are subjected to steam at 212° F. for about 30 minutes, the appearance of the fabric is altered. If the paste is applied in patterns, that portion of the fabric which is thus treated becomes chalky in contrast to the luster of the remaining portions. 30

Terpineol, or camphor oil or other products containing terpineol can be substituted for pine oil, and various starches and gums such as gum arabic can be utilized in preparing the composition. Monopole oil can be replaced by another penetrant and other alkalies can be substituted for caustic soda. 40

Other changes may be made in the details of procedure without departing from the invention or sacrificing any of the advantages thereof. 45

We claim:

1. The method of producing ornamental effects on fabrics including cellulose acetate which comprises imprinting a design on the fabric in a medium including pine oil, and subjecting the fabric before drying to steam at a temperature above 212° F., for a period sufficient to develop the design. 50
2. The method of producing ornamental effects on fabrics including cellulose acetate which 55

comprises imprinting a design on the fabric in a medium including pine oil, and subjecting the fabric before drying to steam for a period sufficient to develop the design.

5. 3. The method of producing ornamental effects on fabrics including cellulose acetate which comprises imprinting a design on the fabric in a medium including a starch, a gum and pine oil

and subjecting the fabric before drying to steam for a period sufficient to develop the design.

4. A composition for producing ornamental effects on fabrics including cellulose acetate, comprising starch, gum tragacanth, water and pine oil.

WINFRED MAXWELL MITCHELL.  
HENRI LOUIS BARTHELEMY.